

## UNITED STATES PATENT OFFICE

2,566,130

## MANUFACTURE OF GLASSINE PAPER

Karl R. Karlson, Evanston, Pa., and Clifford E. Peterson, Finesville, N. J., assignors to Riegel Paper Corporation, New York, N. Y., a corporation of New Jersey

No Drawing. Application June 10, 1944,  
Serial No. 539,787

5 Claims. (Cl. 92—3)

1

This invention relates to the manufacture of glassine and greaseproof paper, etc. and includes an improved method of manufacture and the paper resulting therefrom.

According to the present invention bleached semi-chemical pulps from broad-leaf, short-fibered woods, which pulps contain a large part of the normal hemi-cellulose contents of such woods, are subjected to beating or refining under controlled pH conditions to retain a high proportion of hemi-cellulose in the resulting paper.

The manufacture of glassine and greaseproof papers, etc. is commonly effected by using long-fiber sulfite pulp, such as Mitscherlich pulp, and subjecting it to prolonged refining and beating to effect so-called hydration and with accompanying conversion of the long fibers into shorter fibers to a greater or less extent during the refining and hydrating operation.

The present invention is based upon the discovery that improved greaseproof and glassine papers can be produced from bleached semi-chemical pulp from broad-leaf, short-fibered woods substantially free from lignin and retaining a large proportion of the normal hemi-cellulose content of such woods by subjecting such pulps to refining or beating and hydration with control of the hydrogen ion concentration between about pH 6.0 and pH 9.0 and advantageously between the range of about pH 7.4 and pH 7.8. By such regulation of the pH during the refining and hydrating treatment of the pulp important advantages are obtained both in the refining and hydrating operation and in the resulting greaseproof and glassine papers, etc.

The bleached semi-chemical pulp used in the present process is produced from the wood of broad-leaf trees by subjecting such woods to semi-chemical pulping, e. g., with a neutral or nearly neutral sulfite liquor to soften and dissolve the lignins in the wood chips to permit separation of the fibers by simple attrition. The pulp thus manufactured contains approximately all or most of the hemi-cellulose which is available in the broad-leaf wood. The semi-chemical pulp thus produced by cooking under approximately neutral conditions is distinguished from the pulps produced by the acid and alkali cooking liquors commonly used by its retention of a large proportion of hemi-cellulose which would be largely removed by the acid and alkali cooks.

The semi-chemical pulp contains, in addition to its high hemi-cellulose content, a considerable amount of residual lignin. This is removed from the pulp by a regulated bleaching carried out

2

under approximately neutral conditions, e. g., by multi-stage bleaching with alkali hypochlorite with strict control of pH conditions, temperatures and pressures so that the high hemi-cellulose content is retained in the bleached pulp while the residual lignin is removed.

The resulting bleached pulp will be substantially free from lignin but will contain in addition to the normal celluloses of the wood a large amount of the original hemi-cellulose present in the wood. Advantageously the bleached pulp will contain at least three-quarters of the original hemi-celluloses present in the short-fiber wood from broad-leaf trees. A high hemi-cellulose content results from the semi-chemical pulping and bleaching operations in which strongly acid and alkali liquors are avoided.

The semi-chemical pulping process and also the bleaching are advantageously carried out so that the pulp, both after the pulping process and after the bleaching, remains slightly on the alkaline side, e. g., around a pH of 7.4.

In making the new glassine and greaseproof papers it is important to subject the semi-chemical bleached pulp of high hemi-cellulose content to treatment within a fairly narrow range of conditions and advantageously at a hydrogen ion concentration which does not deviate to any considerable extent from around pH 7.4. Thus the refining of this stock for the making of glassine, greaseproof or similar papers is advantageously controlled so that the hydrogen ion concentration is within the field of about pH 6.0 to pH 9.0. This range is advantageously further restricted between the narrow field of about 7.4 and 7.8 for optimum physical qualities.

According to one embodiment of the invention the bleached, semi-chemical pulp having a pH of about 7.4 is subjected to beating or refining without the addition of any chemicals so that the pulp does not deviate materially from that pH during the beating or refining operation. By maintaining such conditions during beating or refining the desired hydration is obtained with less power consumption than that normally required in making glassine or greaseproof paper from long-fiber sulfite pulp and hydration can be attained with very excellent fibrillation and without any objectionable or excessive cutting of the fibers to attain the desired freeness relation.

The present process can also advantageously be carried out with the addition of metallic compounds and particularly aluminum compounds to the pulp but when such compounds are used care should be taken to control the pH of the

pulp during the beating or hydrating treatment. The use of aluminum compounds tends to produce a more stable bond between the different types of celluloses present and tends to increase the permanency of the bond accomplished in the felting of the fibers. But when aluminum compounds are used in the present process the pH of the pulp is adjusted to avoid acid conditions such as would result from the use of ordinary paper makers' alum. When paper makers' alum is used other salts or compounds should also be used to give the necessary pH control. Thus paper makers' alum can be used together with aluminum hydroxide in proportions which will maintain the desired pH range. So also salts can be used containing the aluminum radical which salts in solution will maintain the pH range within that above indicated. The proportions of the different compounds used will vary somewhat with water conditions, etc., but may be, for example,  $\frac{1}{4}\%$  of aluminum hydroxide with  $\frac{3}{4}\%$  of aluminum sulfate or paper makers' alum, although these proportions may need variation to maintain the pH control above mentioned. Sodium aluminate and paper makers' alum may similarly be used in suitable proportions; or aluminum hydroxide or sodium aluminate may be used with sulfuric or acetic acid in proper proportions.

While the use of aluminum compounds is particularly advantageous for certain kinds of paper, it is possible to use other metallic compounds such as those of zinc, barium, boron, and iron, etc. in the form of soluble salts and with care to keep the pH within the proper range during the beating or refining treatment.

It is one advantage of the present process that the stock can be refined to a freeness far lower than that normally used with long-fiber sulfite pulp. Thus, to make a good No. 1 glassine paper from long-fiber sulfite pulp it is common to refine the stock to a freeness not below 70 cc. and usually around 90 cc. and rarely is the freeness down to 50 cc. (the method of determining freeness is the modified Canadian standard method). Stock lower than 50 cc. freeness is not economical to handle as it would stick to the paper machine wire and to the presses. However, by using the bleached semi-chemical pulp from short-fiber woods according to the process of the present invention the stock can be beaten or otherwise refined down to a freeness of around 20 cc. and good drainage still obtained on the wire without sticking on the presses. In other words, the drainage is still very good even though the slowness is much greater.

In the manufacture of glassine stock from long-fiber sulfite pulp the refining process usually requires the use of stone tackles; but this is not necessary in the process of the present invention to attain the desired improved results from the bleached semi-chemical pulp of high hemi-cellulose content.

Aside from the advantages obtained during the beating or refining and hydrating treatment, such as lower power consumption, decreased freeness etc., other important advantages are obtained in the making of the paper on the paper machine from the refined and hydrated pulp. The drying of the sheet is easier, and it is accompanied with less tendency to cockling, even though the stock is unusually slow. Plasticizing or the inculcation of size or wax emulsions on size presses is very readily done.

The resulting sheets produced by the process

of the present invention are characterized by increased physical strength properties so that, for instance, the bursting test is from 90 to over 100% on the basis weight; total tear by Elmendorf test, totalling the machine and cross-direction, shows around 170 to 225% on the weight basis; the stretch of the sheet, particularly when plasticized with simple sugars, and/or glycerin is 10 to 12%; and the folding endurance on the 10 Schopper folding tester is more than double that of No. 1 glassine available on the market and subjected to test. When the new sheet of the 15 present invention is supercalendered, as in the making of glassine, the sheet is more transparent than the equivalent grade made from other chemical pulp such as long-fiber sulfite.

The greaseproof and glassine papers of the present invention are characterized by a smooth surface and well adapted for printing or writing 20 with a pen even though the sheet is not sized. The greaseproofness of the sheet is equal to or better than similar sheets made from other common pulps such as long-fiber sulfite.

Another advantage of the new paper shown 25 by laboratory tests is that the paper is not influenced by variations in humidity conditions as much as similar papers made from other pulps.

The advantages of the new paper appear to 30 special advantage when the paper are waxed. The waxed sheets retain the desirable qualities of the waxed sulfite sheet without losing the typical glassine qualities. Thus normal waxed glassine paper when crumpled in the hands readily cracks and ruptures in innumerable points of 35 creasing; while the waxed glassine paper of the present invention does not readily rupture under the same treatment.

Another valuable quality of the paper of the present invention as it comes off the paper machine, the supercalender stack, the wlexer, coater, or other converting operation, is a low coefficient 40 of expansion, lower than is normally encountered in similar papers. This is particularly significant considering the slowness of the stock.

It is another advantage of the paper of the present invention that it has improved durability on heat treatment or aging, as compared with similar papers. Papers of improved durability are obtained without the incorporation of aluminum radicals or other metallic radicals as well as when such metallic radicals are incorporated to enhance the durability of the folding and strength development.

The improved paper of the present invention 55 retains a large proportion of the hemi-cellulose content originally present in the short-fiber wood and in the bleached semi-chemical pulp therefrom used in the present process. Thus with broad-leaf woods containing around 20% of hemi-cellulose based on the total cellulose content of the wood a large proportion, advantageously around 13.5% or more, may be retained in the finished paper. The improved properties 60 of the finished paper, whether greaseproof paper or glassine, etc., appear to be due to the high hemi-cellulose content and to its intimate association with the other celluloses of the bleached, semi-chemical pulp. Sheets may thus be readily made which more closely resemble cellophane

65 than greaseproof or glassine paper made by other processes.

It is another advantage of the present invention that it makes possible the production of glassine sheets of lighter weight than can readily be produced from ordinary sulfite pulp but sheets

which are nevertheless characterized by desirable strength and other properties. Sheets may thus be made of e. g., 15-pound weight, this being the weight of 500 sheets 24" by 36".

The paper above described is made entirely from the bleached semi-chemical pulp by subjecting it to the process of the present invention, and such sheets have important advantages, such as those above mentioned.

Composite papers can, however, be made to advantage by combining the refined and hydrated pulp produced by the present process with hydrated and refined pulps produced by other processes. Thus Mitscherlich pulp, after hydrating and refining and with the use of alum during the process, may be washed to remove the alum and to give an approximately neutral pulp and this refined and hydrated pulp then admixed with the hydrated and refined bleached semi-chemical pulp produced by the present process using, e. g., 40 parts of the sulfite pulp and 60 parts of the semi-chemical pulp. These pulps should be hydrated and refined separately and the final mixture of the pulps which is made after the refining should for maximum strength and greaseproofness be kept within the range of pH 6 to 9 and advantageously around pH 7.4. The incorporation of the improved hydrated and refined pulp of the present invention with ordinary sulfite pulp gives a composite sheet of improved physical strength properties.

We claim:

1. The method of producing greaseproof and glassine papers, which comprises subjecting bleached, neutral-sulfite semi-chemical pulp from broad-leaf, short-fiber woods substantially free from lignin and of high hemi-cellulose content to mechanical refining and hydration with regulation of the pH between about 6 and 9 and forming the paper from the resulting refined and hydrated pulp.

2. The method of producing greaseproof and glassine papers, which comprises subjecting bleached, neutral-sulfite semi-chemical pulp from broad-leaf, short-fiber woods substantially free from lignin and of high hemi-cellulose content to mechanical refining and hydration with regulation of the pH at about 7.4 to 7.8.

3. The method of producing greaseproof and glassine papers, which comprises subjecting bleached, neutral-sulfite semi-chemical pulp from broad-leaf, short-fiber woods substantially free from lignin and containing upwards of 10% of hemi-cellulose to mechanical refining and hydration with regulation of the pH between about 6 and 9 and forming the paper from the resulting refined and hydrated pulp.

4. The method of producing greaseproof and glassine papers, which comprises subjecting

bleached, neutral-sulfite semi-chemical pulp from broad-leaf, short-fiber woods substantially free from lignin and containing upwards of 10% of hemi-cellulose to mechanical refining and hydration with regulation of the pH about 7.4 to 7.8 and forming the paper from the resulting refined and hydrated pulp.

5. The method of producing greaseproof and glassine papers, which comprises subjecting bleached, neutral-sulfite semi-chemical pulp from broad-leaf, short-fiber woods substantially free from lignin and of high hemi-cellulose content to mechanical refining and hydration with regulation of the pH between about 6 and 9, separately subjecting long fiber sulfite pulp to mechanical hydrating and refining with the addition of alum, washing the resulting pulp to remove alum and to give an approximately neutral pulp, admixing the resulting refined and hydrated pulp with the hydrated and refined, bleached, neutral-sulfite, semi-chemical pulp to give a mixed pulp of pH between about 6 and 9, and forming the paper from the resulting admixed pulp.

KARL R. KARLSON.  
CLIFFORD E. PETERSON.

#### REFERENCES CITED

The following references are of record in the file of this patent:

#### UNITED STATES PATENTS

| Number       | Name     | Date          |
|--------------|----------|---------------|
| 53,247       | Heaton   | Mar. 13, 1866 |
| 35 1,332,541 | Clapp    | Mar. 2, 1920  |
| 1,631,834    | Schorger | June 7, 1927  |
| 1,648,838    | Barnard  | Nov. 8, 1927  |
| 1,651,665    | Bradley  | Dec. 6, 1927  |
| 1,716,006    | Rinman   | June 4, 1929  |
| 40 1,850,139 | Richter  | Mar. 22, 1932 |
| 1,850,702    | Allen    | Mar. 22, 1932 |

#### FOREIGN PATENTS

| Number     | Country   | Date          |
|------------|-----------|---------------|
| 45 116,594 | Australia | Feb. 16, 1943 |

#### OTHER REFERENCES

- "Chemical Abstracts," vol. 37 (1943), pages 1866, 3601.  
 50 "Manufacture of Pulp and Paper," 3d edition (1938), vol. 4, section 1, page 58.  
 "Paper Industry and Paper World," Oct. 1943, pages 812, 813.  
 "Paper Trade Journal," Nov. 28, 1940, pages 131-134; July 15, 1943, pages 23-25.  
 55 "Technical Association Papers," Series 11 (1928), pages 177-180; Series 20 (1937), page 429; Series 22 (1939), pages 329-332; Series 23 (1940), page 529; and Series 25 (1942), pages 595-599.